

## 1

2,937,978

## ELECTROPLATING OF NICKEL

Wennemar Strauss, Dusseldorf-Holthausen, Alfred Kirstahler, Dusseldorf, Wolfgang Gundel, Dusseldorf-Oberkassel, and Hermann Haas, Dusseldorf-Holthausen, Germany, assignors to Dehydag, Deutsche Hydrierwerke G.m.b.H., Dusseldorf, Germany, a corporation of Germany

No Drawing. Filed July 26, 1955, Ser. No. 524,616

Claims priority, application Germany Aug. 13, 1954

12 Claims. (Cl. 204—49)

This invention relates to an electroplating process, and more particularly to a process of electrodepositing metals from electroplating baths modified with organic sulfonic acids or their salts.

Copending application Ser. No. 442,199, filed July 8, 1954, now Patent No. 2,849,351, describes an electroplating process which employs electroplating baths modified with thioalkane-sulfonic acid compounds having the general structural formula  $Z-S-R-SO_3H$  or their water-soluble salts, wherein Z is a radical comprising a carbon atom directly attached to two atoms selected from the group consisting of nitrogen, sulfur and oxygen atoms, the carbon atom also directly attached to the terminal sulfur atom of the  $-S-R-SO_3H$  group, and R represents a bivalent aliphatic radical which may be unsubstituted or may carry other organic substituent groups, such as ethylene, propylene, alkylpropylene, hydroxy propylene or pentylene groups. Specific examples of such compounds are the following:

N,N - diethyl - dithiocarbamic acid - n - propylester - 1 - sodium sulfonate

2 - mercapto - benzothiazol - S - propane - 1 - sodium sulfonate

Isothiourea-S-propane-1-sodium sulfonate

S-phenyl-trichiocarbonic acid-1-propane-1-sodium sulfonate

Isothiourea-S-butane-1-sodium sulfonate

N,N - pentamethylene - dithiocarbamic acid - n - propyl-ester-1-sodium sulfonate

N,N-dimethyl-dithiocarbamic acid-n-propylester-1-sodium sulfonate

and the like.

In copending application Ser. No. 443,694, now abandoned, filed July 15, 1954, an electroplating process is disclosed which employs electroplating baths modified with organic sulfonic acid compounds having the structural formula



or their water-soluble salts, wherein X represents a halogen, cyano or thiocyanate radical and R represents an aliphatic, cycloaliphatic or aromatic radical which may carry further substituent groups. Specific examples of such compounds are the following:

3-bromopropane-1-sodium sulfonate

4-iodobutane-1-sodium sulfonate

2-bromoethane-1-sodium sulfonate

4-bromobenzene-sodium sulfonate

3-chloropropane-1-sodium sulfonate

3-thiocyanopropane-1-sodium sulfonate

4-thiocyanobutane-1-sodium sulfonate

and the like.

We have found that the characteristics of metal electrodeposits can be improved to an unexpected and surprising degree if the electroplating bath is modified with

## 2

both of the above-described compounds simultaneously. Metal electrodeposits produced from electroplating baths containing both types of sulfonic acid compounds are characterized by considerably greater brightness, much improved distribution of the metal deposit, complete freedom from porosity and absolute uniformity. The high quality metal electrodeposits obtained in this manner can not be produced with electroplating baths modified with only one of the sulfonic acid compounds as disclosed in said copending applications, nor could it have been expected that a combination of these additives in the same electroplating bath would improve the deposits to the degree that it does.

The amounts in which these sulfonic acid compounds are added to the electroplating bath to produce the improved electrodeposits in accordance with the present invention depend largely upon the composition of the bath and the operating conditions, but they generally range between 0.01 and 20 gm. per liter of bath. The temperature range within which such modified baths may be employed with satisfactory results is between 15 and 65° C. The pH-value of the bath may vary between 3.8 and 4.5, and the current density may vary between 0.5 and 12 amp./dm.<sup>2</sup>.

The electroplating baths modified with the two types of sulfonic acid compounds in accordance with this invention, i.e. simultaneously with the thioalkane sulfonic acid derivatives and the halogen-, cyano- or thiocyanato-substituted organic sulfonic acids, may be further modified with known brightening agents, porosity-preventing agents, smoothing agents and wetting agents. For example, known brightening agents which we have found to be particularly advantageous include polyvalent alcohols such as ethylene-glycol, butanediols, glycerin, erythrite, pentaerythrite, sorbitol, sugars, di- or trialkanolamines, also unsaturated alcohols such as butinediol, and furthermore derivatives of polyvalent alcohols which still contain free hydroxyl groups, such as etheralcohols and the like.

Wetting agents which may be advantageously added to the electroplating baths according to our invention are, for example, water-soluble salts of alkylsulfonic acids, alkylarylsulfonic acids, and alkylsulfuric acid esters, or water-soluble ethyleneoxide addition products of fatty alcohols, fatty acids, amines and the like.

In some instances it is also advantageous to add to the electroplating baths inorganic brightening agents in small amounts, such as salts of zinc, cadmium or cobalt.

Metals upon which electrodeposits may be applied with the aid of the baths modified in accordance with the present invention include all those which are ordinarily used for this purpose, such as, for example, iron, steel, zinc and aluminum, metal alloys such as brass, and other suitable non-precious metals.

All common types of electroplating baths may be modified with the sulfonic acid compounds above-disclosed, particularly nickel-plating, copper-plating, zinc-plating, silver-plating and other like electroplating baths.

The following examples will further illustrate our invention and enable others skilled in the art to understand the invention more completely. It is understood, however, that we do not wish to limit our invention to the examples given below.

## Example I

A nickel-plating bath, having a pH of about 4.5 and containing 210 gm. per liter nickel sulfate, 60 gm. per liter nickel chloride and 35 gm. per liter boric acid, was modified by dissolving therein 4 gm. per liter 3-chloropropane-1-sodium sulfonate and 1 gm. per liter isothiourea-S-propane-1-sodium sulfonate. Iron objects were nickel-plated in this bath at a temperature of 45° C. and

a current density of 5 amp./dm.<sup>2</sup>. The nickel electrodeposit produced thereby was of mirror-like brightness and firmly adhered to the iron surfaces of the objects. The brightness and adhering qualities of the nickel deposit produced in this manner were far superior to deposits produced from similar nickel baths under similar conditions of temperature and current density, but modified with only one of the above sulfonic acid compounds.

*Example II*

A nickel-plating bath containing 400 gm. per liter nickel sulfate, 50 gm. per liter nickel chloride and 35 gm. per liter boric acid was modified by adding 10 gm. per liter 3-bromo-propene-1-sodium sulfonate, 0.2 gm. per liter isothiourea-S-propene-1-sodium sulfonate and 5 gm. per liter of glycerin. Sheet steel was then electroplated in this bath. The nickel electrodeposit produced thereby was of exceptionally high brightness and had excellent adhering qualities and ductility.

*Example III*

A nickel-plating bath as described in Example I was modified with 5 gm. per liter 4-iodo-butane-1-sodium sulfonate, 0.5 gm. per liter ethylenethiourea-S-propene-1-sodium sulfonate and 1 gm. per liter butylenediol-1,4. Copper objects which were electroplated in this bath were provided with a nickel plate which was completely free from pores and extremely bright.

*Example IV*

A nickel-plating bath as described in Example II was modified with 6 gm. per liter of 2-bromo-ethane-sodium sulfonate, 0.2 gm. per liter isothiourea-S-propene-1-sodium sulfonate and 8 gm. per liter triethanolamine. Metal objects electroplated in this bath were provided with smooth, extremely bright nickel deposits, which adhered excellently to the metal base and were completely free from pores and uniformly distributed over the entire surface.

*Example V*

The nickel-plating baths described in Examples I and II were modified by dissolving therein 6 gm. per liter of 4-thiocyanato-butane-1-sodium sulfonate, 0.2 gm. per liter isothiourea-S-propene-1-sodium sulfonate and 10 gm. per liter glucose. Iron objects electroplated in these baths were provided with a nickel plate of exceptionally high brightness and smoothness.

While we have given certain specific examples of our invention, we wish it to be understood that the invention is not limited to these examples and that various changes and modifications may be made therein without departing from the spirit of our invention or the scope of the appended claims.

We claim:

1. An electroplating bath for producing bright, non-porous nickel deposits, comprising an acid solution of an inorganic salt of nickel and, as brightening agents, about 0.01 to 20 g. per liter of a compound selected from the group consisting of organic sulfonic acids having the general structural formula



and their water-soluble salts, wherein X is selected from the group consisting of halogen, cyanide and thiocyanide radicals, and R is an aliphatic radical with from 2 to 4 carbon atoms, and about 0.01 to 20 g. per liter of a compound selected from the group consisting of organic sulfonic acids having the general structural formula



and their water-soluble salts, wherein Z is a radical comprising a carbon atom directly attached to two atoms selected from the group consisting of nitrogen, oxygen and sulfur atoms, said carbon atom also directly attached to the terminal sulfur atom of the  $-S-R-SO_3H$  group, 75

and R is a bivalent aliphatic radical with from 3 to 4 carbon atoms.

2. A nickel electroplating bath for producing bright, non-porous nickel deposits, comprising an acid solution of inorganic nickel salts and, as brightening agents, 4 g. per liter of 3-chloropropene-1-sodium sulfonate and 1 g. per liter of isothiourea-S-propene-1-sodium sulfonate.

3. A nickel electroplating bath for producing bright, non-porous nickel deposits, comprising an acid solution of inorganic nickel salts and, as brightening agents, 10 g. per liter of 3-bromopropene-1-sodium sulfonate, 0.2 g. per liter of isothiourea-S-propene-1-sodium sulfonate and 5 g. per liter of glycerin.

4. A nickel electroplating bath for producing bright, non-porous nickel deposits, comprising an acid solution of inorganic nickel salts and, as brightening agents, 5 g. per liter of 4-iodobutane-1-sodium sulfonate, 0.5 g. per liter of ethylenethiourea-S-propene-1-sodium sulfonate and 1 g. per liter of butylenediol-1,4.

5. A nickel electroplating bath for producing bright, non-porous nickel deposits, comprising an acid solution of inorganic nickel salts and, as brightening agents, 2 g. per liter of 2-bromoethane-1-sodium sulfonate, 0.2 g. per liter of isothiourea-S-propene-1-sodium sulfonate and 8 g. per liter of triethanolamine.

6. A nickel electroplating bath for producing bright, non-porous nickel deposits, comprising an acid solution of inorganic nickel salts and, as brightening agents, 6 g. per liter of 4-thiocyanobutane-1-sodium sulfonate, 0.2 g. per liter of isothiourea-S-propene-1-sodium sulfonate and 10 g. per liter of glucose.

7. The process of producing bright, non-porous nickel electrodeposits, which comprises electrodepositing said nickel from a bath containing said nickel principally in the form of an acid solution of an inorganic salt of the nickel in the presence of two brightening agents, one selected from the group consisting of organic sulfonic acids having the general structural formula



and their water-soluble salts, said compounds being present in an amount of about 0.01 to 20 g. per liter, wherein X is selected from the group consisting of halogen, cyanide and thiocyanide radicals, and R is an aliphatic radical with from 2 to 4 carbon atoms, the other selected from the group consisting of organic sulfonic acids having the general structural formula



50 and their water-soluble salts, said compounds being present in an amount of about 0.01 to 20 g. per liter, wherein Z is a radical comprising a carbon atom directly attached to two atoms selected from the group consisting of nitrogen, sulfur and oxygen atoms, said carbon atom also directly attached to the terminal sulfur atom of the  $-S-R-SO_3H$  group, and R is a bivalent aliphatic radical with from 3 to 4 carbon atoms.

8. The process of producing bright, non-porous nickel electrodeposits, which comprises electrodepositing said nickel from a bath containing said nickel principally in the form of an acid solution of an inorganic nickel salt in the presence of 4 g. per liter of 3-chloropropene-1-sodium sulfonate and 1 g. per liter of isothiourea-S-propene-1-sodium sulfonate as brightening agents.

9. The process of producing bright, non-porous nickel electrodeposits, which comprises electrodepositing said nickel from a bath containing said nickel principally in the form of an acid solution of an inorganic nickel salt in the presence of 10 g. per liter of 3-bromopropene-1-sodium sulfonate, 0.2 g. per liter of isothiourea-S-propene-1-sodium sulfonate and 5 g. per liter of glycerin as brightening agents.

10. The process of producing bright, non-porous nickel electrodeposits, which comprises electrodepositing said nickel from a bath containing said nickel principally

in the form on an acid solution of an inorganic nickel salt in the presence of 5 g. per liter of 4-iodobutane-1-sodium sulfonate, 0.5 g. per liter of ethylenethiourea-S-propane-1-sodium sulfonate and 1 g. per liter of butinediol-1,4, as brightening agents.

11. The process of producing bright, non-porous nickel electrodeposits, which comprises electrodepositing said nickel from a bath containing said nickel principally in the form of an acid solution of an inorganic nickel salt in the presence of 2 g. per liter of 2-bromoethane-1-sodium sulfonate, 0.2 g. per liter of isothiourea-S-propane-1-sodium sulfonate and 8 g. per liter of triethanolamine, as brightening agents.

12. The process of producing bright, non-porous nickel electrodeposits, which comprises electrodepositing said 15

nickel from a bath containing said nickel principally in the form of an acid solution of an inorganic nickel salt in the presence of 6 g. per liter of 4-thiocyanobutane-1-sodium sulfonate, 0.2 g. per liter of isothiourea-S-propane-1-sodium sulfonate and 10 g. per liter of glucose, as brightening agents.

## References Cited in the file of this patent

## UNITED STATES PATENTS

|    |           |          |       |                |
|----|-----------|----------|-------|----------------|
| 10 | 1,524,448 | Murphy   | ----- | Jan. 27, 1925  |
|    | 1,642,238 | Gardner  | ----- | Sept. 13, 1927 |
|    | 2,647,866 | Brown    | ----- | Aug. 4, 1953   |
|    | 2,648,627 | Donnelly | ----- | Aug. 11, 1953  |

UNITED STATES PATENT OFFICE  
CERTIFICATE OF CORRECTION

Patent No. 2,937,978

May 24, 1960

Wennemar Strauss et al.

It is hereby certified that error appears in the printed specification of the above numbered patent requiring correction and that the said Letters Patent should read as corrected below.

Column 1, line 40, for "trichiocarbonic" read -- trithiocarbonic --; column 5, line 1, for "on" read -- of --.

Signed and sealed this 29th day of November 1960.

(SEAL)

Attest:

KARL H. AXLINE  
Attesting Officer

ROBERT C. WATSON  
Commissioner of Patents